

# United States Patent Office

2,711,959

Patented June 23, 1955

1

2,711,959

## WELDING STEEL FOR DEVELOPING HIGH SURFACE HARDNESS UNDER IMPACT

William T. De Long, West Manchester Township, York County, and Gustaf A. Ostrom, Paradise Township, York County, Pa., assignors to The McKay Company, Pittsburgh, Pa., a corporation of Pennsylvania

No Drawing. Application November 3, 1954,

Serial No. 466,661

4 Claims. (Cl. 75—128)

This invention relates to welding steel, i. e., steel which can be weld-deposited, which has important improved characteristics. Our improved welding steel is superior to previously existing welding steels in developing surface hardness and has other superior properties.

Austenitic steels of a number of analyses have been used successfully for hard facing applications. The steels suitable for such use, being austenitic or largely so, have a relatively low level of hardness as deposited but have the property of work hardening under impact to higher surface hardness levels which resist wear. The utility of such steels to resist wear therefore depends upon (1) the original hardness level; (2) the speed with which hardness is increased under impact; and (3) the level of increased hardness produced under impact.

An undesirable property in such steels for many applications is the property of deforming or squashing down which the steel undergoes in developing its hardened surface. That property is especially undesirable in applications such as deposits on rail ends, switch frogs, etc., in which the metal should remain standing up in place as it develops its hard surface.

Since the development of the Hadfield manganese steels about 1886 various modified and improved austenitic type steels have been developed and used. They have manifested differing combinations of physical properties and have had utility but they have left much to be desired. There is a crying need for significant improvements in physical properties which will bring about improved performance.

TABLE I  
Prior hard surfacing welding steels

| No.                       | 1       | 2       | 3       |
|---------------------------|---------|---------|---------|
| C (%)                     | .70     | .70     | .50     |
| Cr (%)                    |         | 18      | 18      |
| Mn (%)                    | 14      | 4       | 4       |
| Ni (%)                    | 4       | 9.5     | 9.5     |
| N (%)                     | .05*    | .05*    | .05*    |
| Mo (%)                    |         | 1.5     |         |
| Tensile (lbs./sq. in.)    | 125,000 | 116,000 | 116,000 |
| Yield (lbs./sq. in.)      | 60,000  | 90,000  | 91,000  |
| Elongation (%)            | 45      | 15      | 15      |
| Shrinkage on Impact (in.) | .068    | .050    | .050    |
| Rc Initial                | 13      | 27      | 27      |
| Rc Final                  | 39      | 36      | 36      |

\*Estimated.

2

Table I is a tabulation of the properties of three known alloy steels numbered consecutively from 1 to 3, inclusive. They are typical austenitic type alloy welding steels now widely used for hard surfacing. No. 1, sold under various names including "Hardalloy 118," is a nickel-manganese steel based on the old Hadfield steel analyses (similar steels are being used with molybdenum at the relatively low level of approximately 1% substituted for all of the nickel and with properties rather similar to the nickel-manganese alloys). The physical properties appearing in the table show that the metal is quite soft as deposited with a yield strength of less than half the tensile strength. Under impact the surface hardness of the metal increases. A laboratory test which has been developed for such materials is to subject a standard sample rod to 2500 blows of 25 foot-pounds each. The hardness of the pounded metal is compared with the initial value to show the rate of increase, and the amount of squashing down which has occurred is also measured.

The final hardness shown under the hammer test values would continue to increase, if the test were continued, to a maximum value between 50 and 60 Rc at 80,000 blows. The additional squashing which would occur after the first 2500 blows is negligible as compared with the squashing effected by the first 2500 blows. Under the pounding test (2500 25 foot-pound blows) the "Hardalloy 118" went from a surface hardness of 13 Rc to 39 Rc and at the same time the standard specimen decreased .068" in height.

Steels Nos. 2 and 3 of Table I, sold under the trade names "Frogalloy M" and "Frogalloy C," respectively, are modified 18-8 type austenitic hard facing materials of higher cost than No. 1. Although Nos. 2 and 3 have a little lower tensile strength, they show higher yield strength, higher hardness as deposited and less squashing or shrinkage under the standard pounding test. Because of these properties the "Frogalloy" deposits or closely similar analyses have been considered superior for many hard facing uses. The properties of these modified 18-8 analyses were the best that had been developed in the field of austenitic welding steels for producing hard surfaces prior to the present invention.

We have discovered that superior properties can be developed by the proper balancing of chromium, manganese and nickel coupled with carbon and nitrogen within defined limits, and that further improvement in properties can be obtained by addition of molybdenum and/or tungsten, and/or vanadium and/or columbium within defined limits.

Table II shows the results of tests made with certain improved welding steels which we have developed.

TABLE II  
Improved welding steels

| No.                       | 4       | 5       | 6       | 7       | 8       | 9       |
|---------------------------|---------|---------|---------|---------|---------|---------|
| C (%)                     | .35     | .35     | .30     | .40     | .50     | .40     |
| Cr (%)                    | 20.3    | 12.5    | 16      | 16      | 16      | 16      |
| Mn (%)                    | 12.5    | 16      | 16      | 16      | 16      | 16      |
| Ni (%)                    | 1       | 1       | 1       | 1       | 1       | 1       |
| N (%)                     | .05*    | .05*    | .14     | .15     | .15     | .15     |
| Mo (%)                    | 0       | 0       | 0       | .00     | .2      | .2      |
| V (%)                     | 0       | 0       | 0       | .8      | .8      | .8      |
| Tensile (lbs./sq. in.)    | 134,000 | 115,000 | 130,000 | 144,000 | 152,000 | 144,000 |
| Yield (lbs./sq. in.)      | 93,000  | 78,000  | 97,000  | 117,000 | 120,000 | 121,000 |
| Elongation (%)            | 24      | 44      | 38      | 24      | 23      | 21      |
| Shrinkage on Impact (in.) | .033    | .059    | .054    | .0111   | .021    | .028    |
| Rc Initial                | 27      | 18      | 29      | 31      | 30      | 30      |
| Rc Final                  | 39      | 40      | 34      | 38      | 36      | 40      |

\* Estimated.

Referring to steel No. 6 of Table II, with that analysis pound test values and hardness levels before and after pounding are approximately the same as for the modified 18-8 type (Nos. 2 and 3 of Table I) but the tensile strength, yield strength and elongation are much improved.

Steels Nos. 4 and 5 of Table II, which we developed, are toward the ends of the chromium-manganese area found to be most useful and show that while the properties vary somewhat a high general level is maintained over the ranges evidenced.

To obtain the benefits of our invention the chromium content of the welding steel should be in the range 11-21% while the manganese is in the range 9-19%, and when to this base area of chromium and manganese carbon and alloy additions are made within defined limits combinations of properties are developed which are outstanding. A narrower preferred base area is chromium 14-19% and manganese 14-18%. For example, steels Nos. 7, 8 and 9 of Table II, which we developed, taken as a group show very high tensile and yield strengths, good elongation, good resistance to shrinkage on impact, high initial hardness and good final hardness. Their properties average far beyond those which have been found in the chromium-nickel or austenitic manganese alloys heretofore available. The effect of carbon, chromium, manganese, nickel and alloy additions has been studied extensively to find the approximate limits within which the benefits of our invention are obtained. Table III shows the broad and preferred ranges of elements for accomplishing our improved results.

TABLE III

|                            | Broad Range              | Preferred Range          |
|----------------------------|--------------------------|--------------------------|
| C                          | .20 to .85%.             | .35 to .85%.             |
| Mn                         | 9 to 19%.                | 14 to 18%.               |
| Ni                         | 0 to 4%.                 | 0 to 2%.                 |
| Mn+2Ni                     | 13 to 29%.               | 16 to 22%.               |
| Cr                         | 11 to 21%.               | 14 to 19%.               |
| N                          | 0 to 30%.                | .10 to .25%.             |
| Mo and/or W                | 0 to 5%.                 | 0 to 5%.                 |
| V and/or Cb                | 0 to 2%.                 | 0 to 2%.                 |
| Mo and/or W+2(V and/or Cb) | 10(C-.70) to 10(C+.20)%. | 10(C-.60) to 10(C-.10)%. |

<sup>1</sup> C stands for percent of carbon in the alloy. Only positive values of the parenthetical expressions in this line are significant, negative values are treated as zero.

We have found that two relationships are important. The first is the balance between the austenitizers (C, Mn, Ni, N) and ferritizers (Cr, W, Mo, Cb, V). This balance must be adequate to produce a strong matrix. With all the austenitizers near the low limits of their ranges and the ferritizers near the high limits of their ranges the mechanical properties are little or no better than those of the modified 18-8 type welding steels mentioned above. For this reason limits as to the effective sum of the manganese and the nickel are included in Table III. The total value of manganese plus 2 nickel defines the effect of the two in the alloy in accordance with standard metallurgical practice in relation to austenitic alloys.

The second important relationship is that between carbon and the strong carbide formers (Cr, W, Mo, Cb, V). To illustrate, assume that an optimum balance has been found between the austenitizers and the ferritizers to form a good matrix such as is present in steel No. 6 of Table II; as more strong carbide former is added carbon should be added in small amounts to maintain the alloy balance. Guidance for maintaining the required relationship is given in Table III in which the quantities of molybdenum and/or tungsten, and/or vanadium and/or columbium which may be employed are specified as a function of the carbon content. Carbon and nitrogen exert their usual strong austenitizing action and the carbon range specified is needed to maintain the hardness level and wearing quality developed in the welding steel. In our welding

steel vanadium is approximately twice as powerful as molybdenum. Tungsten and columbium can be substituted respectively for all or part of the molybdenum and vanadium. The limits for molybdenum and/or tungsten plus 2 vanadium and/or columbium are set as a function of the carbon content by positive values of the expressions given; negative values are treated as zero.

With regard to other elements, the austenitizers copper and cobalt may be present in limited quantities. 10 Silicon will normally be present in quantities up to 1.5 or even 2% since it is present in the commercial material available as core wire and is usually used as a deoxidizer in the coatings of coated welding electrodes. Other strong carbide formers such as tantalum or titanium could theoretically be substituted for the carbide formers listed but are hard to recover in weld deposits.

15 The deposit analyses disclosed can be produced by the various methods of manual and automatic welding, as, for example, shielded arc, inert arc, submerged arc or acetylene.

20 While we have described certain present preferred embodiments of the invention it is to be distinctly understood that the invention is not limited thereto but may be otherwise variously embodied within the scope of the 25 following claims.

We claim:

1. A weld deposit which under impact develops high surface hardness without excessive shrinkage having substantially the following composition:

20 C----- .2 to .85%.  
Mn----- 9 to 19%.

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

25

30

in which, in the expressions C-.60 and C-.10, "C" stands for the per cent. of carbon in the welding steel and only positive values of such expressions are significant, negative values being treated as zero; the balance, except for impurities which do not substantially affect the properties of the steel, being iron.

3. An article comprising a structure having welded thereto a deposit which under impact develops high surface hardness without excessive shrinkage having substantially the following composition:

|                      |                          |
|----------------------|--------------------------|
| C-----               | .20 to .85%.             |
| Mn-----              | 9 to 19%.                |
| Ni-----              | 0 to 4%.                 |
| Mn+2Ni-----          | 13 to 22%.               |
| Cr-----              | 11 to 21%.               |
| N-----               | 0 to .30%.               |
| Mo and/or W-----     | 0 to 5%.                 |
| V and/or Cb-----     | 0 to 2%.                 |
| Mo and/or W+2(V and/ |                          |
| or Cb)-----          | 10(C-.70) to 10(C+.20)%. |

in which, in the expressions C-.70 and C+.20, "C" stands for the per cent. of carbon in the welding steel and only positive values of the expression C-.70 are significant, negative values being treated as zero; the balance, except for impurities which do not substantially affect the properties of the steel, being iron.

4. An article comprising a structure having welded

thereto a deposit which under impact develops high surface hardness without excessive shrinkage having substantially the following composition:

|    |                      |                          |
|----|----------------------|--------------------------|
| 5  | C-----               | .35 to .85%.             |
|    | Mn-----              | 14 to 18%.               |
|    | Ni-----              | 0 to 2%.                 |
|    | Mn+2Ni-----          | 16 to 22%.               |
|    | Cr-----              | 14 to 19%.               |
|    | N-----               | .10 to .25%.             |
| 10 | Mo and/or W-----     | 0 to 5%.                 |
|    | V and/or Cb-----     | 0 to 2%.                 |
|    | Mo and/or W+2(V and/ |                          |
|    | or Cb)-----          | 10(C-.60) to 10(C-.10)%. |

15 in which, in the expressions C-.60 and C-.10, "C" stands for the per cent. of carbon in the welding steel and only positive values of such expressions are significant, negative values being treated as zero; the balance, except for impurities which do not substantially affect the properties of the steel, being iron.

References Cited in the file of this patent:

UNITED STATES PATENTS

|    |           |                |              |
|----|-----------|----------------|--------------|
| 25 | 2,671,726 | Jennings ----- | Mar. 9, 1954 |
|    | 2,698,785 | Jennings ----- | Jan. 4, 1955 |

FOREIGN PATENTS

|         |               |               |
|---------|---------------|---------------|
| 152,291 | Austria ----- | Jan. 25, 1938 |
|---------|---------------|---------------|